

T. M. GODFREY.  
OILPROOF AND GREASEPROOF PAPER CAN.  
APPLICATION FILED OCT. 1, 1918.  
1,395,272.

Patented Nov. 1, 1921.

Fig. 1



Fig. 2.



Truman M. Godfrey Inventor  
By his Attorneys  
Pennington, Marvin & Edmunds

# UNITED STATES PATENT OFFICE.

TRUMAN M. GODFREY, OF CHICAGO, ILLINOIS, ASSIGNOR TO THE AMERICAN COTTON OIL COMPANY, OF NEW YORK, N. Y., A CORPORATION OF NEW JERSEY.

## OILPROOF AND GREASEPROOF PAPER CAN.

1,395,272.

Specification of Letters Patent.

Patented Nov. 1, 1921.

Application filed October 1, 1918. Serial No. 256,448.

To all whom it may concern:

Be it known that I, TRUMAN M. GODFREY, a citizen of the United States, residing at Chicago, in the county of Cook, State of Illinois, have invented certain new and useful Improvements in Oilproof and Greaseproof Paper Cans; and I do hereby declare the following to be a full, clear, and exact description of the invention, such as will 5 enable others skilled in the art to which it appertains to make and use the same.

The present invention relates to certain new and useful improvements in paper cans and like containers for substances of an oily 15 or greasy character, and is intended to provide a paper can or container which is made oil-proof or grease-proof by lining it interiorly with a substance which penetrates the paper to some extent and which is flexible 20 (in the sense that it will not crack or check during any normal use to which the can may be subjected), and which is practically odorless and of a nature which will not injure the fat with which it is in contact.

As an example of the application of my 25 invention, I have illustrated in the accompanying drawing, one form of container which is interiorly coated as described in this application. In the drawing,

Figure 1 is an illustration of the container 30 with a portion thereof broken away; and

Fig. 2 is an enlarged detail in section of the wall of the container.

It is to be understood that the illustration 35 is not intended to limit my invention to the particular form of container shown, the invention being equally applicable to other containers within the scope of the accompanying claims.

To this end, the coating consists of an adhesive substance, soluble in water and miscible when in water solution with glycerin, the composition thus made up being of a character to not only adhere to the interior 45 surfaces of the paper container, but also to penetrate and fill the pores of the paper for a sufficient distance to anchor the resulting lining in place, while leaving a substantial body of the material as a surface film covering the entire periphery that is to be exposed to the oil or grease. Furthermore, when set, the coating forms a continuous film or layer of the coating material over the 50 inner periphery of the container so as to ex-

clude the penetration of the oil or grease into 55 the body portion of the protected paper.

In the practical carrying out of the invention, the adhesive employed may be, for instance, gum arabic, dextrin, glue or gelatin, casein or the like, associated with water and 60 glycerin, to which, when casein is employed, a proportion of ammonium hydrate may be added.

When gum arabic is employed as the adhesive, it will be suitable to employ 50 parts 65 by weight of gum arabic, 135 parts by weight of water and 25 parts by weight of glycerin; this solution should be applied warm, for the reason that it penetrates more readily and is somewhat more fluid when warm. 70

When dextrin is employed as the adhesive it will be suitable to employ 200 parts by weight of dextrin, 150 parts by weight of water, and 40 parts by weight of glycerin. When glue or gelatin is employed as the adhesive, it will be suitable to employ 10 parts by weight of glue or gelatin, 42 parts by weight of water and 7 parts by weight of glycerin. When casein is employed as the adhesive, it will be suitable to employ 10 80 parts by weight of casein, 100 parts by weight of water, 10 parts by weight of glycerin, and to add from 5 to 10 parts by weight of ammonium hydrate ( $\text{NH}_4\text{OH}$ ) of a specific gravity of 0.90. 85

It will, of course be understood that the proportions of these various constituents may vary somewhat without materially affecting the grease-proof properties of the solution. In practice, it will be found appropriate and in many instances necessary to apply two coats of any of these solutions, for the reason that there are apt to be small air bubbles, resulting in minute or pin-hole openings in a single coat which would permit the oil or grease to slowly leak through, whereas the application of a second coating will compensate for this defect by filling the openings referred to. 90

It will be of particular advantage, in many 100 instances, to make up the oil-proof and grease-proof coating, by first applying to the interior of the paper container the casein solution, and, when this first coating is sufficiently dry, to then apply a second coating 105 of either the gum arabic solution or the gelatin solution. The advantage of this combination is that the casein coating produces a

much whiter finish upon the paper (even though it be a poor grade of paper) than would the gum arabic solution or the gelatin solution if used alone, while the use of the 5 gum arabic solution or the gelatin solution to form a top coating makes it possible to use a lower grade casein without any objectionable odor being noticeable. So also, since the use of a first coating of casein upon the 10 paper produces an excellent white finish, it is feasible to use a lower grade of paper for the can than could be used to advantage if a gum arabic solution or a gelatin solution were employed as the sole coating.

15 Referring to the drawing, 5 indicates a container which, in the present instance, is cylindrical in form and is provided with a cap or closure 6. The container is constructed of paper and may, for example, be provided with double walls 7 which are suitably secured together. The exact form and construction of the container forms no part of my present invention, which, as above indicated relates to the coating thereof to render 20 the paper impervious to substances of an oily or greasy character. The coating 8 is of the character above described and is applied in any suitable manner to accomplish the desired purpose.

It is a characteristic merit of the coatings hereinbefore described that, in contradistinction to like coatings omitting glycerin, they are of a tough, consistent, and flexible character, exhibiting no tendency to crack, chip, or check, in the normal use to which the 35 containers are put and, at the same time, being entirely oil and grease-proof, so that, particularly, they may serve as receptacles for edible products of an oily or greasy character, such as edible vegetable and animal oils and greases, both of liquid and non-liquid consistency, for which employment they are notably adapted.

What I claim is:

A paper container having an inner coating produced by the application thereto first of glycerin, water, and casein, and secondly, of glycerin, water and an adhesive soluble in water and of a character to mask any objectionable odor of the casein employed in 50 the first coating; substantially as and for the purposes described.

In testimony whereof I affix my signature.

TRUMAN M. GODFREY.

Witnesses:

JOHN C. MYERS,  
L. V. JENKINS.